

Feb. 13, 1973

KAZUO MATSUDO ET AL

3,716,420

HOT ROLLED STEEL SHEETS FOR EXTRA DEEP DRAWING

Filed Nov. 8, 1971

2 Sheets-Sheet 1



Feb. 13, 1973

KAZUO MATSUDO ET AL

3,716,420

HOT ROLLED STEEL SHEETS FOR EXTRA DEEP DRAWING

Filed Nov. 8, 1971

2 Sheets-Sheet 2

*FIG. 2*



*FIG. 3*



**3,716,420**  
**HOT ROLLED STEEL SHEETS FOR EXTRA**  
**DEEP DRAWING**

**DEEP DRAWING**

Kazuo Matsudo, Koichi Osawa, and Yoshisuke Ikegami,  
Fukuyama, Japan, assignors to Nippon Kokan Kabu-  
shiki Kaisha

Filed Nov. 8, 1971, Ser. No. 196,697  
Claims priority, application Japan, Dec. 19, 1970,  
45/113,660

Int. Cl. C21d 1/74, 9/48 10  
U.S. Cl. 148—12 3 Claims

## ABSTRACT OF THE DISCLOSURE

A hot rolled steel sheet having extra deep drawing and press formability properties comparable to cold rolled steel sheets, wherein the steel is vacuum degassed and has a composition consisting essentially of: 0.001-0.020% carbon, less than 0.10% silicon, 0.10-0.60% manganese, less than 0.020% sulphur, 0.010-0.10% aluminum, 0.02-0.08% titanium, balance iron and incidental impurities and wherein  $Ti/C < 4$  and  $Ti/S > 2$ . The steel sheets are hot rolled with a finishing temperature in the range 800-950° C. and coiled at a temperature in the range 650° C.-700° C. 15 20 25

This invention relates to steel sheets and in particular to hot rolled steel sheets having a relatively low tensile strength and excellent press formability.

Heretofore most extra deep drawing steels are produced by cold rolling processes, but such processes are relatively expensive. It is, therefore, economically advantageous to provide hot rolled sheets for drawing purposes provided press formability equal to that of cold rolled sheets can be achieved in sheets in the range of 1.6–3.4 mm. thick. For example, a 3.2 mm. thick sheet produced by cold rolling has an approximate notch elongation of 20% but by conventional hot rolling for drawing the notch elongation falls far short of that level.

It is, therefore, an object of the present invention to provide a hot rolled steel sheet having a notch elongation of at least 20%.

A number of proposals have been made concerning provision of hot rolled steel sheets having excellent press formability. Notable among these are vacuum degassed aluminum killed steels and desulfurized low manganese aluminum killed steels. Table 1 shows an example of each of the two types of prior art hot rolled steels together with the heat treatments and mechanical properties of such steels.

Applicants have found that similar or superior properties can be achieved in hot rolled steel sheets of 1.0-7.0 mm. thick provided such steels, are vacuum degassed and contain a carefully controlled addition of titanium. 5

Thus, by one aspect of the present invention there is provided a steel consisting essentially of 0.001-0.020% carbon, less than 0.10% silicon, 0.10-0.60% manganese, less than 0.020% sulphur, 0.010-0.10% aluminum, 0.02-0.08% titanium, balance iron and incidental impurities, provided always that  $Ti/C < 4$  and  $Ti/S > 2$ .

By a preferred embodiment the steel of the present invention is hot rolled at a finishing temperature between 800-950° C. and coiled at a temperature between 650-700° C.

Specific reasons for limiting the quantity of the components of the hot rolled steel sheets of this invention are explained in more detail hereafter.

Increases in carbon content cause increases in carbide precipitation which are in turn detrimental to the press formability of the steel. In the steel of the present invention, therefore, the carbon content is reduced as much as

TABLE 1

| Items                         | Composition (percent) by weight |      |      |       |       |        | Thickness of sheets, mm. | Finishing temperature, °C. | Colling temperature, °C. | Direction, C. | YP, kg./mm. <sup>2</sup> | TS, kg./mm. <sup>2</sup> | EI, percent | Mechanical property | EIN, percent |      |
|-------------------------------|---------------------------------|------|------|-------|-------|--------|--------------------------|----------------------------|--------------------------|---------------|--------------------------|--------------------------|-------------|---------------------|--------------|------|
|                               | C                               | Si   | Mn   | P     | S     | Ni     |                          |                            |                          |               |                          |                          |             |                     |              |      |
| Degassed Al killed steel      | 0.01                            | Tr.  | 0.32 | 0.018 | 0.017 | 0.0029 | 0.043                    | 3.2                        | 900                      | 680           | [L]<br>[C]               | 21.2                     | 31.2        | 50.4                | 0            | 18.0 |
| Degassed Al killed steel      | 0.04                            | 0.01 | 0.18 | 0.010 | 0.012 | 0.0030 | 0.016                    | 3.2                        | 870                      | 665           | [L]<br>[C]               | 21.5                     | 31.4        | 50.7                | 0.2          | 17.0 |
| Degsl. low Mn Al killed steel | 0.04                            | 0.01 | 0.18 | 0.010 | 0.012 | 0.0030 | 0.016                    | 3.2                        | 870                      | 665           | [L]<br>[C]               | 25.6                     | 32.1        | 51.5                | 2.8          | 19.4 |
| Degsl. low Mn Al killed steel | 0.04                            | 0.01 | 0.18 | 0.010 | 0.012 | 0.0030 | 0.016                    | 3.2                        | 870                      | 665           | [L]<br>[C]               | 25.6                     | 32.5        | 52.1                | 6.0          | 19.1 |

NOTE.—EIN represents notch elongation in a notch tensile test which furnishes a reliable standard for evaluating press formability of thin sheets.

possible by vacuum degassing so as to achieve higher press formability. 0.001% carbon is the practical lower limit of decarbonization by vacuum degassing and the upper limit of 0.020 represents the point above which the tensile strength of the steel rises sharply because of TiC precipitation.

Silicon is another element which increases the tensile strength of steel sheets and therefore this element is restricted to amounts below 0.1%.

Manganese in an amount in excess of 0.1% is added in order to prevent hot shortness caused by sulphur. The upper limit of manganese must, however, be controlled to less than 0.6% because manganese works, like carbon and silicon, to increase the tensile strength of the steel.

Sulphur is maintained at a level of less than 0.020% because larger amounts affect the cleanliness of the steel and adversely affect the press formability because of the formation of MnS.

Titanium is added to the steel because it converts MnS from an A type to a C type impurity. An A type inclusion or impurity is defined as one which is plastically deformed by working, and a C type inclusion is defined as one which

cause press formability rises proportionately as the coiling temperature increases, it is preferred that the coiling temperature should lie between 650° C.-700° C. An example of this invention is set forth below:

5

#### EXAMPLE 1

Table 2 indicates the chemical composition of steels covered by this invention and Table 3 indicates the manufacturing conditions and mechanical properties upon hot rolling of such steels.

TABLE 2

|                | Percent by weight |
|----------------|-------------------|
| C              | 0.008             |
| Si             | Tr.               |
| 15 Mn          | 0.20              |
| P              | 0.011             |
| S              | 0.012             |
| N <sub>2</sub> | 0.0040            |
| Sol Al         | 0.035             |
| 20 Ti          | 0.03              |
| Ti/C           | 3.7               |
| Ti/S           | 2.5               |

TABLE 3

| Thickness of plates<br>(mm.) | Hot rolling<br>conditions (°C.) |                             |                             | Skin-<br>pass,<br>percent | Test<br>direc-<br>tion | Mechanical property         |                |                  |                 |                             |   |
|------------------------------|---------------------------------|-----------------------------|-----------------------------|---------------------------|------------------------|-----------------------------|----------------|------------------|-----------------|-----------------------------|---|
|                              | Finishing<br>temper-<br>ature   | Cooling<br>temper-<br>ature | YP,<br>kg./mm. <sup>2</sup> |                           |                        | TS,<br>kg./mm. <sup>2</sup> | El,<br>percent | YPEl,<br>percent | ElN,<br>percent | AI,<br>kg./mm. <sup>2</sup> |   |
| 3.2                          | 890                             | 680                         | 1.0                         | 1.0                       | L<br>C                 | 17.8<br>18.0                | 30.0<br>30.5   | 52.9<br>51.8     | 0<br>0          | 22.7<br>22.4                | 0 |

NOTE : AI=Aging index.

is scattered at random throughout the matrix and which is not plastically defined by working. The C type inclusion is less detrimental to press formability, and at the same time produces solid solution of sulphur to some extent through the formation of TiN thereby serving to decrease MnS-type sulfides extending in the direction of rolling. Thus, the Ti added to hot rolled steel sheets achieve excellent press formability. It has been found that the Ti content must satisfy the ratio Ti/S>2 in order to achieve the above noted conditions. In addition, the ratio Ti/C<4 further serves to improve the press formability of the hot rolled steel sheets provided the condition of Ti/S>2 is also met. For the above reasons, the Ti content is fixed at 0.02-0.08% bearing in mind its further balance with the carbon and sulphur contents.

Aluminum is added in an amount of 0.010%-0.10% in order to facilitate deoxidation and effect a better Ti yield. Amounts in excess of 0.10% are detrimental to the press formability of the steel sheets, and an amount less than 0.010% lessens the effect of deoxidation.

In order to achieve the desired mechanical properties in the hot rolled steel sheets for extra deep drawing, the heat treatment steps must be controlled within the temperature ranges previously discussed.

In order to produce steel sheets for extra deep drawing having excellent press formability, it is desirable that finishing temperature of the rolling is above the Ar<sub>3</sub> transformation temperature, because the press formability rapidly deteriorates below the Ar<sub>3</sub> temperature. However, the Ar<sub>3</sub> transformation temperature is in the vicinity of 850° C. in the case of sheets of extremely low carbon content and it is difficult to maintain a finishing temperature as high as 850° C. in very thin sheets. However, the effect of a finishing temperature below the Ar<sub>3</sub> transformation temperature is, at least in part, offset by careful control of the steel composition within the ranges previously discussed. Because the steels of the present invention range from 1.0 to 7.0 mm. thick, the range of finishing temperatures may be between 800° C. and 950° C. In operations, it is desirable to maintain a finishing temperature as high as possible above the Ar<sub>3</sub> transformation temperature. On the other hand, the coiling temperature can be less than 650° C. and still provide an acceptable press formability. Be-

35 As is clear from this example, steels manufactured in accordance with this invention have low tensile strength and excellent press formability.

In order to more clearly illustrate the differences between the steels of the present invention and other hot rolled steel sheets for drawing of the same thickness, reference is made to the accompanying drawings in which:

40 FIG. 1 shows the relation between the notch elongation percentage and the tensile strength respectively of the products of the present invention and the prior art.

FIG. 2 is a microphotograph (100 magnifications) of the structure of a steel plate manufactured by the method of this invention and

45 FIG. 3 is a microphotograph (500 magnifications) of the structure of inclusions.

Differences in notch elongation between steels of this invention and other hot rolled steel sheets for drawing of the same thickness are shown in FIG. 1. It is obvious therefrom that the press formability of the steel sheets of this invention is far superior to those of the conventional hot rolled steel sheets for drawing, an approach is that of cold rolled steel sheets.

50 As shown in FIG. 2, the microphotograph of the ferrite structure of a steel sheet according to this invention shows an ideal formation. FIG. 3 shows that Al<sub>2</sub>O<sub>3</sub> and MnS are closely attached to TiN+TiS. This gain shows that excellent characteristics may be achieved by products of the present invention.

The embodiments of the invention in which an exclusive property or privilege is claimed are defined as follows:

55 1. A vacuum degassed steel hot rolled into sheets for extra deep drawing, said steel consisting essentially of: 0.001-0.020% carbon, less than 0.10% silicon, 0.10-0.60% manganese, less than 0.020% sulphur, 0.010-0.10% aluminum, 0.02-0.08% titanium, balance iron and incidental impurities and wherein Ti/C<4 and Ti/S>2.

60 2. A steel sheet as claimed in claim 1 wherein said sheet is hot rolled with a finishing temperature within the range of 800-950° C. and coiled at a temperature in the range of 650-700° C. whereby press formability properties are enhanced.

3. A process for producing steel sheets for extra deep drawing, comprising vacuum degassing a steel having a composition consisting essentially of 0.001-0.020% carbon, less than 0.10% silicon, 0.10-0.60% manganese, less than 0.020% sulphur, 0.010-0.10% aluminum, 0.02-0.08% titanium, balance iron and incidental impurities and wherein  $Ti/C < 4$  and  $Ti/S > 2$ , hot rolling said steel into sheets 1.0-7.0 mm. thick with a rolling finishing temperature in the range of 800-950° C. and coiling said steel sheet at a temperature in the range 650-700° C.

## References Cited

## UNITED STATES PATENTS

|             |        |                       |        |
|-------------|--------|-----------------------|--------|
| 3,522,110   | 7/1970 | Shimizu et al. -----  | 148-12 |
| 3,560,270   | 2/1971 | Reinbold et al. ----- | 148-12 |
| 5 3,607,456 | 9/1971 | Forand, Jr. -----     | 148-12 |

WAYLAND W. STALLARD, Primary Examiner

U.S. Cl. X.R.

10 148-12.1, 36